

May 15, 1962

R. F. POWELL ET AL

3,034,648

PROMOTING FROTH FLOTATION

Filed April 29, 1959

5 Sheets-Sheet 1



Fig. 1.

R. F. POWELL  
E. F. MARTIN  
J. LURIE  
R. J. NICHOL  
E. M. BRAND  
*Inventors*

By  
Wendewirth, Lind & Ponack Attorneys

May 15, 1962

R. F. POWELL ET AL

3,034,648

PROMOTING FROTH FLOTATION

Filed April 29, 1959

5 Sheets-Sheet 2



Fig. 2.

R. F. POWELL  
E. F. MARTIN  
J. LURIE  
R. J. NICHOL  
E. M. BRAND  
*Inventors*

By  
Wendover, Lind & Ponack Attorneys

May 15, 1962

R. F. POWELL ET AL

3,034,648

PROMOTING FROTH FLOTATION

Filed April 29, 1959

5 Sheets-Sheet 3



Fig. 3.

R. F. POWELL  
E. F. MARTIN  
J. LURIE  
R. J. NICHOL  
E. M. BRAND  
*Inventors*

By  
Wenderoth, Lind & Ponack Attorneys

May 15, 1962

R. F. POWELL ET AL

3,034,648

PROMOTING FROTH FLOTATION

Filed April 29, 1959

5 Sheets-Sheet 4



Fig. 4.

R. F. POWELL  
E. F. MARTIN  
J. LURIE  
R. J. NICHOL  
E. M. BRAND  
*Inventors*

By  
Wenderoth, Lind & Ponack Attorneys

May 15, 1962

R. F. POWELL ET AL

3,034,648

PROMOTING FROTH FLOTATION

Filed April 29, 1959

5 Sheets-Sheet 5



Fig. 5.

R.F. POWELL  
E.F. MARTIN  
J. LURIE  
R.J. NICHOL  
E.M. BRAND  
*Inventors*

By

Wenderoth, Lind & Ponack Attorneys

## 1

3,034,648

### PROMOTING FROTH FLOTATION

Roger Frederick Powell, Johannesburg, Eric Francis Martin, Germiston, Julian Lurie and Robert James Nichol, Johannesburg, and Ernst Marais Brand, Pretoria, Union of South Africa, assignors to National Chemical Products Limited, Germiston, Union of South Africa, a company of the Union of South Africa

Filed Apr. 29, 1959, Ser. No. 809,814

Claims priority, application Union of South Africa  
May 9, 1958

8 Claims. (Cl. 209—166)

This invention relates to the use of new chemical compounds as accelerators in the froth flotation of mineral ore.

The new chemical compounds have the general formula:



wherein  $\text{R}_1$ ,  $\text{R}_2$  and  $\text{R}_3$  are alkoxy-substituted straight chain alkyl radicals in which the straight chain portion has 1 to 3 carbon atoms and the alkoxy substituent also has 1 to 3 carbon atoms.

The process for producing these new chemical compounds comprises polymerising, in the presence of catalytic quantities of a halogen, one or more substituted aldehydes having 2 to 4 carbon atoms and each containing as a substituent an alkoxy group having 1 to 3 carbon atoms. Depending on whether or not the starting material is a single substance or a mixture of these substances  $\text{R}_1$ ,  $\text{R}_2$  and  $\text{R}_3$ , in the general formula above, may be the same or different. Iodine is the preferred catalyst.

The novel substances of this invention are shown by examples given in detail hereafter to have valuable properties in the art of flotation, when used additionally to known promoters such as xanthates, with or without known frothers being also present; as the more detailed examples show, their net effect is to "accelerate" the flotation in a concentrate of the particular mineral being floated by the known promoters and frothers. As is well-known in the art of flotation the effect of a particular reagent differs from ore to ore and it is therefore well-known to test by standardised well-known procedures the effect both in degree and kind of a particular reagent on a particular ore.

The new chemical compounds of this invention may with some ores show a dominance of their collecting properties and with other ores a dominance of their frothing properties and the degree of effectiveness of the said properties will also depend on the particular ore being used. Furthermore the new compounds of this invention can either be used in their purified form or can be used directly as the reaction product of the reactions set out hereunder by way of example, without purification.

As a method of identification the infra-red spectra of a

## 2

number of these compounds were obtained and are set out in the drawings annexed thereto in which:

FIG. 1 is the infra-red absorption spectrum of 2,4,6-tris-(2' methoxypropyl)-1,3,5-trioxane.

5 FIG. 2 is the infra-red spectrum of the beta-methoxypropionaldehyde polymer. The sample from which this spectrum was prepared was not quite pure, the impurities showing up in e.g. the absorption at about 2.75 and 5.75 microns;

10 FIG. 3 is the infra-red spectrum of the beta-ethoxybutyraldehyde polymer;

FIG. 4 is the infra-red spectrum of the beta-n-propoxybutyraldehyde polymer;

15 FIG. 5 is the infra-red spectrum of the copolymer of beta-methoxybutyraldehyde and beta-ethoxybutyraldehyde referred to below.

Other identifying properties of these substances are given in Table I below.

20 Purely by way of example and without in any way limiting the generality of the foregoing some examples will now be given for the purpose of illustrating this invention.

### EXAMPLE I

#### Production of 2,4,6-Tris-(2' Methoxy-Propyl)-1,3,5-Trioxane

25 200 mls. of beta-methoxybutyraldehyde having a water content of less than 0.1% and preferably less than 0.05% is treated with 0.1 gm. of iodine. Heat is liberated and 30 the temperature rises from about room temperature to about 50° C. in approximately 10 minutes. However, it has been noticed that the reaction may continue slowly after this stage.

At the completion of the vigorous reaction or, if desired, some time thereafter, the reaction product is purified by distillation in known manner to yield the above-mentioned new chemical substance which has a boiling point of 100° C. at 0.05 mm. mercury. The structural formula of this substance is:



### EXAMPLE II

55 Other members of the class of new chemical compounds according to this invention can be prepared in a manner similar to Example I. Further examples are therefore given below of the production of other representative members of this class. These examples are arranged in the order of the starting materials, i.e. the substituted aldehydes, giving first the processes and thereafter giving the identifying properties of the compounds produced.



Table II

| Product          | Percent Weight | Copper            |                              |                                            | Zinc              |                              |                                            | Sulphur         |                             |                                           |
|------------------|----------------|-------------------|------------------------------|--------------------------------------------|-------------------|------------------------------|--------------------------------------------|-----------------|-----------------------------|-------------------------------------------|
|                  |                | Assay, Percent Cu | Percent Wt. X Assay Units Cu | Percent Recovery Units Cu Percent of Total | Assay, Percent Zn | Percent Wt. X Assay Units Zn | Percent Recovery Units Zn Percent of Total | Assay Percent S | Percent Wt. X Assay Units S | Percent Recovery Units S Percent of Total |
| Con A            | 7.23           | 7.24              | 52.34                        | 41.4                                       | 7.87              | 56.90                        | 13.7                                       | 23.19           | 167.7                       | 11.6                                      |
| Con B            | 7.34           | 3.79              | 27.82                        | 22.0                                       | 11.73             | 86.10                        | 20.7                                       | 18.16           | 133.3                       | 9.2                                       |
| Con C            | 6.48           | 2.69              | 17.43                        | 13.9                                       | 25.29             | 163.88                       | 39.4                                       | 22.69           | 147.0                       | 10.1                                      |
| Con D            | 22.12          | 1.17              | 25.88                        | 20.5                                       | 4.04              | 89.36                        | 21.4                                       | 29.81           | 880.6                       | 60.8                                      |
| Cumulative Cons. | 43.17          | -----             | 128.47                       | 97.8                                       | -----             | 296.24                       | 95.2                                       | -----           | 1,328.6                     | 91.7                                      |
| Tails            | 56.83          | 0.05              | 2.85                         | 2.2                                        | 0.35              | 19.89                        | 4.8                                        | 2.12            | 120.5                       | 8.3                                       |
| Calc. Heads      | 100            | 1.26              | 126.32                       | 100                                        | 4.16              | 146.13                       | 100                                        | 14.49           | 1,449.1                     | 100                                       |

Table III

|                     | Substituted Aldehyde Polymerized                                       | Chemical Name of Polymer                                             | Number of Carbon Atoms in    |                            | Structural Formula of R <sub>1</sub> , R <sub>2</sub> , R <sub>3</sub>                                                                                                                               |
|---------------------|------------------------------------------------------------------------|----------------------------------------------------------------------|------------------------------|----------------------------|------------------------------------------------------------------------------------------------------------------------------------------------------------------------------------------------------|
|                     |                                                                        |                                                                      | Straight Chain Alkyl Radical | Alkoxy Substituent Thereon |                                                                                                                                                                                                      |
| M.P.A. Polymer      | Beta-methoxypropionaldehyde.                                           | 2.4.6 - tris - (2' - methoxyethyl)-1.3.5-trioxane.                   | 2                            | 1                          | R <sub>1</sub> , R <sub>2</sub> , R <sub>3</sub> are CH <sub>3</sub> O-CH <sub>2</sub> -CH <sub>2</sub> -                                                                                            |
| E.P.A. Polymer      | Beta-ethoxypropionaldehyde.                                            | 2.4.6 - tris - (2' ethoxyethyl)-1.3.5-trioxane.                      | 2                            | 2                          | R <sub>1</sub> , R <sub>2</sub> , R <sub>3</sub> are C <sub>2</sub> H <sub>5</sub> O-CH <sub>2</sub> -CH <sub>2</sub> -                                                                              |
| P.P.A. Polymer      | Beta-n-propoxypropionaldehyde.                                         | 2.4.6 - tris (2' propoxyethyl)-1.3.5-trioxane.                       | 2                            | 3                          | R <sub>1</sub> , R <sub>2</sub> , R <sub>3</sub> are C <sub>3</sub> H <sub>7</sub> O-CH <sub>2</sub> -CH <sub>2</sub> -                                                                              |
| M.B.A. Polymer      | Beta-methoxybutyraldehyde.                                             | 2.4.6 - tris - (2' methoxypropyl)-1.3.5-trioxane.                    | 3                            | 1                          | R <sub>1</sub> , R <sub>2</sub> , R <sub>3</sub> are CH <sub>3</sub> -CH-CH <sub>2</sub> -<br> <br>OCH <sub>3</sub>                                                                                  |
| M. (E) B.A. Polymer | 2 moles Beta-methoxybutyraldehyde and 1 mole Beta-ethoxybutyraldehyde. | 2.4 - bis - (2' methoxypropyl)-6 - (2' ethoxypropyl)-1.3.5-trioxane. | 3                            | 1 and 2                    | R <sub>1</sub> , R <sub>3</sub> are CH <sub>3</sub> -CH-CH <sub>2</sub> -<br> <br>OCH <sub>3</sub><br>R <sub>2</sub> is CH <sub>3</sub> -CH-CH <sub>2</sub> -<br> <br>OC <sub>2</sub> H <sub>5</sub> |
| E.B.A. Polymer      | Beta-ethoxybutyraldehyde.                                              | 2.4.6 - tris - (2' ethoxypropyl)-1.3.5-trioxane.                     | 3                            | 2                          | R <sub>1</sub> , R <sub>2</sub> , R <sub>3</sub> are CH <sub>3</sub> -CH-CH <sub>2</sub> -<br> <br>OC <sub>2</sub> H <sub>5</sub>                                                                    |
| P.B.A. Polymer      | Beta-n-propoxybutyraldehyde.                                           | 2.4.6 - tris - (2' propoxypropyl)-1.3.5-trioxane.                    | 3                            | 3                          | R <sub>1</sub> , R <sub>2</sub> , R <sub>3</sub> are CH <sub>3</sub> -CH-CH <sub>2</sub> -<br> <br>OC <sub>2</sub> H <sub>7</sub>                                                                    |
| M.A.A. Polymer      | Methoxyacetaldehyde.                                                   | 2.4.6 - tris - (methoxy-methyl)-1.3.5-trioxane.                      | 1                            | 1                          | R <sub>1</sub> , R <sub>2</sub> , R <sub>3</sub> are CH <sub>3</sub> O-CH <sub>2</sub> -                                                                                                             |

Table IV

SUMMARISED RESULTS—PERCENT WEIGHTS  
[Cum = Cumulative]

|                          | Copper Concentrate (Concentrate A) | Copper-Zinc Middlings Concentrate B) | A+B Cum. | Zinc Concentrate (Concentrate C) | A+B+C Cum. | Pyrites Concentrate (Concentrate D) | A+B+C+D Cum. |
|--------------------------|------------------------------------|--------------------------------------|----------|----------------------------------|------------|-------------------------------------|--------------|
| Control                  | 7.23                               | 7.34                                 | 14.57    | 6.48                             | 21.05      | 22.12                               | 43.17        |
| With M.P.A. Polymer      | 8.92                               | 11.82                                | 20.74    | 9.36                             | 30.10      | 20.23                               | 50.33        |
| With E.P.A. Polymer      | 6.82                               | 14.72                                | 21.54    | 10.16                            | 31.70      | 19.20                               | 50.90        |
| With P.P.A. Polymer      | 7.53                               | 13.67                                | 21.20    | 7.77                             | 28.97      | 20.13                               | 27.10        |
| With M.B.A. Polymer      | 9.66                               | 19.50                                | 29.16    | 7.85                             | 37.01      | 17.75                               | 54.76        |
| With M. (E) B.A. Polymer | 7.50                               | 18.50                                | 26.00    | 7.40                             | 33.40      | 18.73                               | 52.13        |
| With E.B.A. Polymer      | 10.00                              | 17.06                                | 27.06    | 8.04                             | 35.10      | 18.24                               | 53.34        |
| With P.B.A. Polymer      | 7.02                               | 14.24                                | 21.26    | 9.07                             | 30.33      | 21.23                               | 51.56        |

## PERCENT RECOVERIES—COPPER

|                         | Copper Concentrate (Concentrate A) | Copper-Zinc Middlings (Concentrate B) | A+B Cum. | Zinc Concentrate (Concentrate C) | A+B+C Cum. | Pyrites Concentrate (Concentrate D) | A+B+C+D Cum. | Calc: Heads Cu., percent |
|-------------------------|------------------------------------|---------------------------------------|----------|----------------------------------|------------|-------------------------------------|--------------|--------------------------|
| Control                 | 41.4                               | 22.0                                  | 63.4     | 13.9                             | 77.3       | 20.5                                | 97.8         | 1.26                     |
| With M.P.A. Polymer     | 55.4                               | 22.1                                  | 77.5     | 12.6                             | 90.1       | 8.8                                 | 98.9         | 1.39                     |
| With E.P.A. Polymer     | 36.8                               | 29.5                                  | 66.3     | 20.0                             | 36.3       | 11.3                                | 97.6         | 1.18                     |
| With P.P.A. Polymer     | 45.0                               | 26.9                                  | 71.9     | 14.5                             | 86.4       | 13.1                                | 99.5         | 1.21                     |
| With M.B.A. Polymer     | 58.7                               | 23.6                                  | 82.3     | 9.4                              | 91.7       | 6.9                                 | 98.6         | 1.17                     |
| With M. (E)B.A. Polymer | 38.6                               | 35.0                                  | 73.6     | 10.7                             | 84.3       | 11.8                                | 96.1         | 1.27                     |
| With E.B.A. Polymer     | 49.1                               | 26.8                                  | 75.9     | 10.8                             | 86.7       | 10.0                                | 96.7         | 1.29                     |
| With P.B.A. Polymer     | 36.3                               | 25.2                                  | 61.5     | 16.7                             | 78.2       | 18.8                                | 97.0         | 1.32                     |

## PERCENT RECOVERIES—ZINC

|                         | Copper Concentrate (Concentrate A) | Copper-Zinc Middlings (Concentrate B) | A+B Cum. | Zinc Concentrate (Concentrate C) | A+B+C Cum. | Pyrites Concentrate (Concentrate D) | A+B+C+D Cum. | Calc: Heads Zinc, percent |
|-------------------------|------------------------------------|---------------------------------------|----------|----------------------------------|------------|-------------------------------------|--------------|---------------------------|
| Control                 | 13.7                               | 20.7                                  | 34.4     | 39.4                             | 73.8       | 21.4                                | 95.2         | 4.16                      |
| With M.P.A. Polymer     | 18.8                               | 29.4                                  | 48.2     | 40.2                             | 88.2       | 8.5                                 | 96.7         | 4.02                      |
| With E.P.A. Polymer     | 14.3                               | 36.3                                  | 50.6     | 39.7                             | 90.3       | 6.8                                 | 97.1         | 3.96                      |
| With P.P.A. Polymer     | 14.5                               | 26.3                                  | 40.8     | 43.8                             | 84.6       | 11.8                                | 98.4         | 3.98                      |
| With M.B.A. Polymer     | 18.9                               | 38.5                                  | 57.4     | 34.4                             | 91.8       | 5.3                                 | 97.1         | 4.00                      |
| With M. (E)B.A. Polymer | 14.1                               | 34.1                                  | 48.2     | 39.7                             | 87.9       | 8.1                                 | 96.0         | 3.87                      |
| With E.B.A. Polymer     | 18.7                               | 34.6                                  | 53.3     | 36.2                             | 89.5       | 6.8                                 | 96.3         | 3.81                      |
| With P.B.A. Polymer     | 14.3                               | 24.0                                  | 38.3     | 45.0                             | 83.3       | 12.7                                | 96.0         | 4.10                      |

## PERCENT RECOVERIES—SULPHUR

|                         | Copper Concentrate (Concentrate A) | Copper-Zinc Middlings (Concentrate B) | A+B Cum. | Zinc Concentrate (Concentrate C) | A+B+C Cum. | Pyrites Concentrate (Concentrate D) | A+B+C+D Cum. | Calc: Heads sulfur, percent |
|-------------------------|------------------------------------|---------------------------------------|----------|----------------------------------|------------|-------------------------------------|--------------|-----------------------------|
| Control                 | 11.6                               | 9.2                                   | 20.8     | 10.1                             | 30.9       | 60.8                                | 91.7         | 14.49                       |
| With M.P.A. Polymer     | 14.5                               | 14.8                                  | 29.3     | 15.6                             | 44.9       | 51.0                                | 95.9         | 14.52                       |
| With E.P.A. Polymer     | 9.5                                | 16.8                                  | 26.3     | 18.0                             | 44.3       | 49.8                                | 94.1         | 14.70                       |
| With P.P.A. Polymer     | 14.3                               | 16.2                                  | 30.5     | 13.1                             | 43.6       | 51.5                                | 95.1         | 14.81                       |
| With M.B.A. Polymer     | 16.2                               | 22.0                                  | 38.2     | 13.1                             | 51.3       | 45.2                                | 98.5         | 14.41                       |
| With M. (E)B.A. Polymer | 11.5                               | 22.1                                  | 33.6     | 11.6                             | 45.2       | 50.3                                | 95.5         | 14.61                       |
| With E.B.A. Polymer     | 16.2                               | 20.3                                  | 36.5     | 12.3                             | 48.8       | 46.5                                | 95.3         | 14.50                       |
| With P.B.A. Polymer     | 10.2                               | 16.2                                  | 26.4     | 16.1                             | 42.5       | 52.4                                | 94.9         | 14.09                       |

These tabulated results will demonstrate clearly to a person-in-the-art the accelerating properties of these new chemical compounds on flotation processes. However, by way of example an analysis is given below of the effects of one of the polymers, namely, "M.B.A. polymer" compared to the control without polymers.

Note, firstly, that for only 2.43% extra weight, 17.3% extra copper is recovered in the "copper pull" (Con. A), but only 5.2% extra zinc; in the "copper-zinc-middlings pull" (Con. B), a relatively large increase of 12.16% extra weight recovers only 1.6% extra copper, but 17.8% extra zinc; in the "zinc-pull" (Con. C), a small increase of 1.37% extra weight recovers 4.5% less copper (because progressively 18.9% extra copper had already been recovered in Cons. A+B), and 5.0% less zinc (because progressively 23.0% extra zinc had ready been recovered in Cons. A+B).

Looking at the other end of the series of operations, the final bulk concentrate of high-grade pyrites (Con. D) was 4.37% less in weight, but contained in it was 13.6% less of the copper, and 16.1% less of the zinc.

The overall loss of copper in the tailings was 0.8% less, and of zinc 1.9% less.

These results clearly demonstrate the characteristic effect of using these chemicals as additives, all other reagents and procedures being identical. This effect is a speeding-up or acceleration of flotation of the particular mineral for whose flotation conditions are correct.

Those skilled in the art will be able to devise plant procedures that make the best use of such effects to give improved metallurgical results.

## EXAMPLE IV

As an illustration of the observed effects obtained by using the new chemical compounds of this invention as accelerators in flotation processes a report is set out in this 50 example of a preliminary test using the M.B.A. polymer in addition to normal promotor and frother on a gold bearing arsено-pyrite ore-concentrating plant.

A feature of the plant was a unit cell included in the grinding circuit, and as it was felt that this would be an 55 ideal place to observe the effects, the accelerator was added to the pump sump immediately before the unit cell.

It was observed that the froth texture and depth changed 60 immediately, becoming much tougher, also showing signs of intense mineral flocculation. As the froth became tougher it appeared that considerable coarser material was being retained and in addition that more slimed graphite and arsено-pyrite was being lifted at this stage.

The rate of addition of accelerator was increased from 65 about 0.1 lb. per ton ore to about double, and instead of "running" the froth became tougher still, the mineral building up to an extent that additional frother (T.E.B/ Pine Oil) and promotor Aerofloat 25 had to be used to get the froth moving.

70 It appeared at this stage that the grade was down slightly but by the amount of material removed the recovery must have increased.

Once this section had settled down, a second reagent 75 feeder was set up over the conditioner to the roughing bank and additional accelerator added at this point.

Similar effects were noticed—bubble texture changed to a smaller more persistent bubble, and the froth toughened up. The load consisted of some fairly coarse material and much slimed graphite and arseno-pyrite.

It was this slimed graphite and arseno-pyrite that gave the most interesting picture. The colour of the cells became much darker than before and the scavengers much lighter in colour, this latter being most unusual. In other words the more sluggish material was coming "up cell" and its rate of flotation increased i.e. "accelerated."

#### EXAMPLE V

This example will illustrate that although certain of the new compounds of this invention e.g. M.B.A. polymer, which from Examples III and IV above is clearly an excellent accelerator, do act as very good frothers in water, nevertheless the accelerating properties of the new compounds of this invention are not necessarily dependent on their ability to form a froth in water.

The following tests were conducted in a Denver-Fahrenwald machine of 10 litre capacity.

30 drops ( $\pm 0.27$  ml.) of unreacted beta-methoxybutyraldehyde were added to 10 litres of water, and upon aeration very little froth was formed.

However, in a comparative test the addition of as little as 2 to 4 drops (0.018 to 0.036 ml.) of the M.B.A. polymer gave, upon aeration, copious volumes of froth of a desirable type. These tests demonstrated water frothing powers of these 2 materials.

A similar test with unreacted beta-ethoxy-butylaldehyde required over 20 drops (0.18 ml.) to give, upon aeration, an appreciable volume of froth, whereas as little as 4 drops (0.036 ml.) of the E.B.A. polymer gave, upon aeration, copious volumes of froth of a desirable type.

The M.A.A. polymer however is completely water soluble and has no visible effect on the water in the standard water frothing test. Nevertheless, when submitted to the ore tests according to Example III it clearly showed the accelerating effect as will be apparent from Table V below in which the results are set out in the same manner as in Table IV above.

Table V  
PERCENT WEIGHTS

|                          | Con A | Con B | A+B Cum. | Con C | A+B+C Cum. | Con D | A+B+C+D Cum. |
|--------------------------|-------|-------|----------|-------|------------|-------|--------------|
| Control.....             | 3.3   | 3.4   | 6.7      | 4.1   | 10.8       | 23.6  | 34.4         |
| With M.A.A. Polymer..... | 4.8   | 5.1   | 9.9      | 6.8   | 16.7       | 25.2  | 41.9         |

PERCENT RECOVERIES COPPER

|                          | Con A | Con B | A+B Cum. | Con C | A+B+C Cum. | Con D | A+B+C+D Cum. | Calc: Heads Cu, percent |
|--------------------------|-------|-------|----------|-------|------------|-------|--------------|-------------------------|
| Control.....             | 29.2  | 21.1  | 50.3     | 11.7  | 62.0       | 36.0  | 98.0         | 1.25                    |
| With M.A.A. Polymer..... | 36.0  | 20.3  | 56.3     | 12.0  | 68.3       | 28.1  | 96.4         | 1.37                    |

PERCENT RECOVERIES ZINC

|                          | Con A | Con B | A+B Cum. | Con C | A+B+C Cum. | Con D | A+B+C+D Cum. | Calc: Heads Zn, percent |
|--------------------------|-------|-------|----------|-------|------------|-------|--------------|-------------------------|
| Control.....             | 8.2   | 9.7   | 17.9     | 32.4  | 50.3       | 43.8  | 94.1         | 3.98                    |
| With M.A.A. Polymer..... | 11.2  | 13.6  | 24.8     | 47.0  | 71.8       | 24.6  | 96.4         | 3.98                    |

PERCENT RECOVERIES SULPHUR

|                          | Con A | Con B | A+B Cum. | Con C | A+B+C Cum. | Con D | A+B+C+D Cum. | Calc: Heads S, percent |
|--------------------------|-------|-------|----------|-------|------------|-------|--------------|------------------------|
| Control.....             | 5.6   | 5.8   | 11.4     | 7.5   | 18.9       | 66.9  | 85.8         | 14.60                  |
| With M.A.A. Polymer..... | 8.9   | 8.5   | 17.4     | 11.4  | 28.8       | 66.3  | 95.1         | 14.62                  |

#### EXAMPLE VI

Reagents E.B.A. Polymer and M.B.A. Polymer Versus Control With T.E.B./Pine Oil on a Barberton Pyrite Ore, pH 8.0

A Denver-Fahrenwald machine of 10 litre capacity was used with an aqueous ore pulp in the manner known to persons skilled in the art. "Starvation" quantities used, 0.018 lb./ton of ore, to pull a concentrate for 5 minutes. Sodium sec.-butylxanthate used as a promotor.

M.B.A. Polymer—74.7% of pyrites floated @ grade 30.46% S.

E.B.A. Polymer—80.6% of pyrites floated @ grade 32.96% S.

"Control"—64.9% of pyrites floated @ grade 36.35% S.

Far the best depth of froth was given by M.B.A. polymer. In the case of E.B.A. polymer and M.B.A. polymer mineral-collecting power was evident, as well as powerful frothing effects.

#### EXAMPLE VII

Reagent M.B.A. Polymer Versus Control With "37 X" (a blend of Triethoxybutane and Triethoxyhexane) on Pyrites-Gold-Bearing Residues From Cyanidation, pH 5.8

(Sodium sec-butylxanthate used as promotor)

A Denver-Fahrenwald machine of 10 litre capacity was used with an aqueous ore pulp in the manner known to persons skilled in the art: 0.040 lb./ton of residues of M.B.A. polymer floated 6.80% weight of concentrates containing 86.9% of the pyrites, and 50.0% of the gold. 0.040 lb./ton of residues of "37 X," floated 5.94% weight of concentrates containing 86.6% of the pyrites, and 48.0% of the gold. In this test the frothing power of M.B.A. polymer was predominant.

**11**  
**EXAMPLE VIII**

*Reagents M.B.A. Polymer and E.B.A. Polymer plus T.E.B./Pine Oil Versus Control With T.E.B./Pine Oil Alone, on a Transvaal Ore Containing Arseno-pyrite and Gold (0.9% As: 12 dwts. Au) pH 7.2*

A Denver-Fahrenwald machine of 10 litre capacity was used with an aqueous ore pulp in the manner known to persons skilled in the art.

In these tests neither M.B.A. polymer nor E.B.A. polymer had any true frothing properties: froths had to be produced by means of the T.E.B./Pine Oil mixture whether or not the M.B.A. polymer or E.B.A. polymer was added.

In each test 0.3 lb./ton of sec-butylxanthate was added at the start, plus the requisite number of drops of T.E.B./Pine Oil frother.

After pulling the first concentrate for 2 minutes, another 0.1 lb./ton of xanthate, and the appropriate quantity of T.E.B./Pine Oil was added; a second concentrate was pulled for 2 minutes.

Then another 0.1 lb. of xanthate, and the appropriate quantity of T.E.B./Pine Oil was added, and a final concentrate pulled for 3 minutes.

*Percentage Recoveries*

**Control:**

56.8% of the As and 65.9% of the Au in first concentrate  
63.2% of the As and 70.4% of the Au in first and second concentrates  
84.9% of the As and 91.5% of the Au in total concentrates

**M.B.A. Polymer 0.048 lb./ton ore additionally:**

85.9% of the As and 89.0% of the Au in first concentrates  
90.0% of the As and 92.4% of the Au in first and second concentrates  
91.6% of the As and 93.8% of the Au in total concentrates

**E.B.A. Polymer 0.048 lb./ton ore additionally:**

77.4% of the As and 83.1% of the Au in first concentrate  
85.1% of the As and 90.8% of the Au in first and second concentrates  
87.5% of the As and 93.0% of the Au in total concentrates

5

10

15

20

25

30

35

40

45

**12**

What is claimed is:

1. In froth flotation of mineral ore with the aid of a promoter, the addition to the froth flotation medium of a compound of the formula



wherein  $\text{R}_1$ ,  $\text{R}_2$  and  $\text{R}_3$  are alkoxy-substituted straight chain alkyl radicals in which the straight chain has from 1 to 3 carbon atoms and the alkoxy substituent also has from 1 to 3 carbon atoms.

2. A process according to claim 1 wherein the said compound is 2,4,6-tris-(2' methoxypropyl)-1,3,5-trioxane.

3. A process according to claim 1 wherein the said compound is 2,4,6-tris-(2' ethoxypropyl)-1,3,5-trioxane.

4. A process according to claim 1 wherein the said compound is 2,4,6-tris-(2' propoxypropyl)-1,3,5-trioxane.

5. A process according to claim 1 wherein the said compound is 2,4,6-tris-(2' methoxyethyl)-1,3,5-trioxane.

6. A process according to claim 1 wherein the said compound is 2,4-bis-(2' methoxypropyl)-6-(2' ethoxypropyl)-1,3,5-trioxane.

7. A process according to claim 1 wherein the said compound is 2,4,6-tris-(methoxymethyl)-1,3,5-trioxane.

8. A process according to claim 1 wherein the said compound is 2,4,6-tris-(ethoxymethyl)-1,3,5-trioxane.

**References Cited in the file of this patent**

**UNITED STATES PATENTS**

|           |           |       |                |
|-----------|-----------|-------|----------------|
| 2,347,447 | Walker    | ----- | Apr. 25, 1944  |
| 2,465,489 | Sokol     | ----- | Mar. 29, 1949  |
| 2,561,251 | Van Aardt | ----- | July 17, 1951  |
| 2,770,654 | Trapp     | ----- | Nov. 13, 1956  |
| 2,901,107 | Fischer   | ----- | Aug. 25, 1959  |
| 2,904,177 | Michal    | ----- | Sept. 15, 1959 |

**OTHER REFERENCES**

Trioxane, Walker and Carlisle, Chemical and Engineering News, volume 21, number 15, August 10, 1943, pages 1250 and 1251.